

# UNITED STATES PATENT OFFICE.

CHARLES SCHWARTZ, OF VILLEURBANNE, FRANCE, ASSIGNOR TO SOCIÉTÉ GILLET & FILS, OF LYON, RHÔNE, FRANCE, A CORPORATION OF FRANCE.

## PROCESS FOR THE TREATMENT OF VEGETABLE FIBERS.

1,400,380.

Specification of Letters Patent. Patented Dec. 13, 1921.

No Drawing.

Application filed December 9, 1919. Serial No. 343,577.

To all whom it may concern:

Be it known that I, CHARLES SCHWARTZ, a citizen of the Republic of France, and a resident of Villeurbanne, Department of

5 Rhône, France, have invented a new and useful Process for the Treatment of Vegetable Fibers, of which the following is a specification.

This invention relates to a process for the 10 treatment of vegetable fibers, with a view more especially to imparting to them the character of wool.

In my patent application No. 343,576 filed herewith, I have described such a process for 15 the treatment of vegetable fibers, of all kinds and in all forms, the process consisting in impregnating the textile material with a solution of cellulose in concentrated nitric acid, preferably of a concentration 20 equal to or higher than 65 per cent., and precipitating upon the textile material a slightly nitrated cellulose, by subjecting the textile material saturated with the solution to an action of washing with water, or to 25 treatment with dilute solutions of acids, bases or salts, followed by washing with water.

It has now been found that an analogous result can be obtained by utilizing instead 30 of cellulose or its products, substances having a constitution approaching that of cellulose, namely starch and in general the amylose products.

The products resulting from the action of 35 the concentrated nitric acid, preferably of a concentration equal to or higher than 65 per cent., upon the starch and amylose substances in general, may be precipitated upon the vegetable fibers either by washing with 40 water, or by treatment with dilute solutions of acids, bases or salts, followed by washing with water.

As in the case of the above mentioned process of patent application No. 343,576 45 of December 9, 1919, there may be employed dilute solutions of acids or bases or saline solutions, for example 10 per cent. aqueous solutions of sulfuric acid, ammonia, ammonium sulfate, sodium bi-sulfate, sodium 50 phosphate and the like. This preliminary treatment, before washing by means of water, renders the precipitation of the nitrated amylose product upon the fibers more rapid and complete.

In order to effect this fixation of the nitrated amylose products upon the vegetable fibers, two different methods of procedure may be adopted.

The textile material may be impregnated with a solution of starch or of an amylose compound in concentrated nitric acid, and the precipitation of the nitrated amylose compound upon the textile effected by the washing with water, or by the treatment with weak alkalis or acids or aqueous solutions of salts, followed by washing with water.

Alternatively, the fibers may be loaded or dressed by means of a solution or paste of starch or other amylose compound, the textile dried and then treated with concentrated nitric acid, the excess of nitric acid pressed out, and the material finally washed; in this case the nitrated amylose product is formed directly upon and in the fiber and absorbed by the latter; it is then definitely precipitated upon and in the same by washing with water, or by treatment with weak alkalis or acids or aqueous solutions of salts, followed by washing with water. This method of procedure presents great advantages, from the point of view of simplicity and convenience of working; textile materials dressed and loaded with a paste in this manner keep indefinitely, they can be prepared long in advance, and be subjected as required to the further treatments with concentrated nitric acid and precipitation of the nitrated amylose product upon the fiber.

The duration of the action and the temperature vary according to the nature of the fibers to be treated, and also according to the amylose substance employed; in general, the time of the soaking of the textile material in the solution of amylose substance in concentrated nitric acid or of the textile dressed with the paste in the concentrated nitric acid, requires to be several minutes and the temperature may vary from 5° C. below zero up to 20° C. above zero, without exerting any appreciable effect upon the final result, just as in the process of my prior patent application No. 343,576 of December 9, 1919.

The process herein described is applicable, like that of my prior application mentioned, to vegetable fibers of all kinds, mercerized

or not, and at any stage whatever in the 5 operation to which they are subjected in the textile industry, whether in the mass or in the form of lap, yarn or fabrics made therewith, and whether these fabrics are fine or coarse, smooth, figured or worked.

The present process allows also of producing 10 figured or damask effects upon plain fabrics; this result can be obtained in various ways. For example the fabrics may be printed at the desired parts with a solution 15 of an amyloseous substance in concentrated nitric acid, or the entire fabric may be impregnated with this solution after printing thereon of suitable resists or reserves at the parts where the production of the effect is not desired; in both cases the excess of acid is pressed out, and the material washed with water, or treated with dilute solutions of 20 acids, alkalis or salts and washed with water, with a view to fixing a precipitate of the nitrated amyloseous product upon the parts impregnated with the solution.

Alternatively the following method may 25 be followed: The fabric is printed, only at the parts where it is desired to produce the figured effect, with an aqueous solution of paste of starch or other amyloseous substances, or again the whole fabric is impregnated, after printing thereon with suitable reserves, with this solution or paste; in either case, the fabric is then passed into concentrated nitric acid, the excess of acid is pressed out, and the nitrated amyloseous 30 product is precipitated and fixed upon the fiber, either by washing by water or by treatment with dilute solutions of acids, alkalis or bases, followed by washing with water.

40 Example: A paste is prepared by heating together 40 kilograms of maize starch, 75 liters of water and 75 liters of acetic acid. The textile is dressed with this paste, dried, treated for 3 to 5 minutes with 72 per cent. 45 nitric acid at a temperature of 15 to 20° centigrade; the excess of acid is pressed out, and the textile material is passed into a 10 per cent. solution of sodium bisulfate and washed with water.

50 The process of the present invention communicates to vegetable fibers the character of wool; the fibers or fabrics increase in weight, become denser and stronger and are softer to the touch; their affinity and ab-

sorbent capacity as regards dyestuffs are 55 considerably increased, even as to basic dyes.

These fibers or fabrics thus transformed may be further treated in any desired manner, in particular they may be dyed, without the new properties acquired being in 60 any way diminished.

Having now particularly described and ascertained the nature of my said invention, and in what manner the same is to be performed, I declare that what I claim is: 65

1. A process for the treatment of vegetable fiber with a view of imparting to it the character of wool, both physically as to feel, appearance and caloric quality, and chemically as regards its affinity and absorbent 70 quality for dyestuffs, said process comprising precipitating upon the fiber the product resulting from the action of concentrated nitric acid upon an amyloseous substance. 75

2. A process for the treatment of vegetable fiber with a view of imparting to it the character of wool, both physically as to feel, appearance and caloric quality, and chemically as regards its affinity and absorbent 80 quality for dyestuffs, said process comprising precipitating upon the fiber the product resulting from the action of nitric acid at a concentration of at least 65% upon an amyloseous substance. 85

3. A process for the treatment of vegetable fibers, for the purpose described, consisting in impregnating the fiber with a solution of an amyloseous substance, drying the fiber, passing the same into concentrated 90 nitric acid, and precipitating the nitrated amyloseous substance upon the fiber by washing. 95

4. A process for the treatment of vegetable fibers, for the purpose described, consisting in impregnating the fiber with a solution of an amyloseous substance, drying the fiber, passing the same into concentrated nitric acid, of a concentration of at least 65%, and precipitating the nitrated amyloseous substance upon the fiber by washing. 100

In testimony whereof I have signed my name to this specification.

CHARLES SCHWARTZ.

Witnesses:

PHILIPPE DESGRANGES,  
WOLFE BOHN.